



US006815081B1

(12) **United States Patent**  
Bremser

(10) **Patent No.:** **US 6,815,081 B1**  
(45) **Date of Patent:** **Nov. 9, 2004**

(54) **COLORING AND/OR EFFECT-CREATING  
MULTILAYER ENAMEL COATING,  
METHOD FOR THE PRODUCTION  
THEREOF AND ITS USE**

(75) Inventor: **Wolfgang Bremser**, Munster (DE)

(73) Assignee: **BASF Coatings AG**, Munster (DE)

(\*) Notice: Subject to any disclaimer, the term of this patent is extended or adjusted under 35 U.S.C. 154(b) by 342 days.

(21) Appl. No.: **10/018,350**

(22) PCT Filed: **Jun. 23, 2000**

(86) PCT No.: **PCT/EP00/05825**

§ 371 (c)(1),  
(2), (4) Date: **Mar. 20, 2002**

(87) PCT Pub. No.: **WO01/02102**

PCT Pub. Date: **Jan. 11, 2001**

(30) **Foreign Application Priority Data**

Jun. 30, 1999 (DE) ..... 199 30 066

(51) **Int. Cl. 7** ..... **B32B 27/32**

(52) **U.S. Cl.** ..... **428/515; 428/516; 428/520;  
428/522; 428/523; 525/64; 525/273; 525/391;  
427/407.1; 427/409**

(58) **Field of Search** ..... **525/64, 273, 391;  
428/522, 520, 515, 516, 523; 427/409,  
407.1**

(56) **References Cited**

U.S. PATENT DOCUMENTS

|             |         |                   |                 |
|-------------|---------|-------------------|-----------------|
| 3,552,986 A | 1/1971  | Bassemir          | ..... 117/12    |
| 3,577,476 A | 5/1971  | Gurney            | ..... 260/668   |
| 4,085,168 A | 4/1978  | Milkovich et al.  | ..... 260/886   |
| 4,413,036 A | 11/1983 | Drexler et al.    | ..... 428/458   |
| 4,521,580 A | 6/1985  | Turner et al.     | ..... 526/307   |
| 4,533,701 A | 8/1985  | Kusumoto et al.   | ..... 525/370   |
| 4,636,545 A | 1/1987  | König et al.      | ..... 524/457   |
| 4,656,226 A | 4/1987  | Hutchins et al.   | ..... 525/93    |
| 4,677,003 A | 6/1987  | Redlich et al.    | ..... 427/373   |
| 5,047,454 A | 9/1991  | Cowles et al.     | ..... 523/500   |
| 5,126,393 A | 6/1992  | Blum et al.       | ..... 524/538   |
| 5,322,715 A | 6/1994  | Jouck et al.      | ..... 427/409   |
| 5,385,996 A | 1/1995  | Rizzardo et al.   | ..... 526/240   |
| 5,395,903 A | 3/1995  | Charmot et al.    | ..... 526/220   |
| 5,516,559 A | 5/1996  | Röckrath et al.   | ..... 427/407   |
| 5,521,229 A | 5/1996  | Lu et al.         | ..... 522/40    |
| 5,565,508 A | 10/1996 | Hoenel et al.     | ..... 523/414   |
| 5,601,880 A | 2/1997  | Schwarze et al.   | ..... 427/407.1 |
| 5,670,557 A | 9/1997  | Dietz et al.      | ..... 522/184   |
| 5,773,543 A | 6/1998  | Rizzardo et al.   | ..... 526/215   |
| 5,830,927 A | 11/1998 | Vanderhoff et al. | ..... 522/81    |
| 5,830,928 A | 11/1998 | Faler et al.      | ..... 523/502   |
| 5,840,372 A | 11/1998 | Rink et al.       |                 |
| 5,854,353 A | 12/1998 | Knoll et al.      | ..... 525/314   |
| 5,857,998 A | 1/1999  | Barry             | ..... 604/96    |
| 5,859,112 A | 1/1999  | Overbeck et al.   | ..... 524/460   |
| 5,905,132 A | 5/1999  | Wegner et al.     | ..... 528/45    |
| 5,959,026 A | 9/1999  | Abusleme et al.   | ..... 524/758   |
| 5,969,030 A | 10/1999 | Grandhee          | ..... 524/457   |

(List continued on next page.)

FOREIGN PATENT DOCUMENTS

|    |           |         |                   |
|----|-----------|---------|-------------------|
| CA | 2004988   | 12/1989 | ..... C08F/2/24   |
| CA | 2103595   | 1/1992  | ..... C08F/2/38   |
| CA | 2086156   | 12/1992 | ..... C09D/175/04 |
| CA | 2127919   | 7/1994  | ..... C08L/57/00  |
| CA | 2181934   | 7/1996  | ..... C08F/282/00 |
| CA | 2259559   | 3/1997  | ..... C08F/8/34   |
| CA | 2205030   | 9/1997  | ..... C08F/2/38   |
| CA | 2355620   | 12/1999 | ..... C08F/293/00 |
| DE | 35 46 594 | 12/1992 | ..... C08F/212/06 |
| EP | 3582211   | 9/1989  | ..... C09D/5/44   |
| EP | 401565    | 5/1990  | ..... C09D/5/02   |
| EP | 498583    | 1/1992  | ..... B01J/19/18  |
| EP | 732359    | 3/1996  | ..... C08K/5/00   |
| EP | 755946    | 7/1996  | ..... C08F/2/22   |
| WO | WO9615157 | 5/1923  | ..... C08F/2/38   |
| WO | WO9106535 | 5/1991  | ..... C07C/409/16 |
| WO | WO9213903 | 8/1992  | ..... C08F/2/38   |
| WO | WO9222355 | 12/1992 | ..... A63B/37/12  |
| WO | WO9322351 | 11/1993 | ..... C08F/2/42   |
| WO | WO9801478 | 1/1998  | ..... C98F/2/38   |
| WO | WO9837104 | 8/1998  | ..... C08F/2/48   |
| WO | WO9910413 | 3/1999  | ..... C08J/3/00   |
| WO | WO9915597 | 4/1999  | ..... C09D/133/00 |

OTHER PUBLICATIONS

Bartol, et al., 09/263,426, Mar. 5, 1999.

Rink et al., 09/830,694, filed Apr. 27, 2003.

Meiseburg, et al., 09/926,532, filed Nov. 16, 2001.

Mangels, et al., 10/088,376, filed Mar. 11, 2002.

Nickolaus et al., 10/250,586, filed Jul. 2, 2003.

Ramesh, et al., 10/455,066, filed Jun. 5, 2003.

Baumgart, et al., 10/049,656, filed Feb. 13, 2002.

(List continued on next page.)

Primary Examiner—D. Lawrence Tarazano

(57) **ABSTRACT**

A multicoat color and/or effect coating system ML for a primed or an unprimed substrate comprising—lying above one another—(1) a surfacer coat FL which absorbs mechanical energy, and (2) a color and/or effect topcoat DL, or (1) a surfacer coat FL which absorbs mechanical energy, (2) a color and/or effect basecoat BL, and (3) a clearcoat KL, or (1) a color and/or effect basecoat BL and (2) a clearcoat KL, wherein at least one coat, preferably at least two coats, and in particular all coats of the multicoat system ML has or have been produced from a coating material comprising at least one constituent (A) preparable by free-radical polymerization of

a) olefinically unsaturated monomers and

b) olefinically unsaturated monomers I different than the olefinically unsaturated monomers (a):

$R^1R^2C=CR^3R^4$  (I),

in which the radicals  $R^1$ ,  $R^2$ ,  $R^3$  and  $R^4$  each independently of one another are hydrogen atoms or alkyl, cycloalkyl, alkylcycloalkyl, cycloalkylalkyl, aryl, alkylaryl, cycloalkylaryl, arylalkyl or arylcycloalkyl radicals, with the proviso that at least two are aryl, arylalkyl or arylcycloalkyl radicals; in an aqueous medium.

24 Claims, No Drawings

## U.S. PATENT DOCUMENTS

|                   |         |                        |            |
|-------------------|---------|------------------------|------------|
| 5,972,809 A       | 10/1999 | Faler et al. ....      | 442/103    |
| 5,990,221 A       | 11/1999 | Dames et al. ....      | 524/457    |
| 6,020,438 A       | 2/2000  | Lubnin et al. ....     | 525/317    |
| 6,046,259 A       | 4/2000  | Das et al. ....        | 524/40     |
| 6,100,350 A       | 8/2000  | Wilczek et al. ....    | 526/82     |
| 6,140,386 A       | 10/2000 | Vanderhoff et al. .... | 522/78     |
| 6,160,049 A       | 12/2000 | Mathauer et al. ....   | 524/804    |
| 6,162,886 A       | 12/2000 | Bremer et al. ....     | 526/318.42 |
| 6,221,949 B1      | 4/2001  | Gross et al. ....      | 524/451    |
| 6,235,857 B1      | 5/2001  | Rizzardo et al. ....   | 526/220    |
| 6,346,591 B1      | 2/2002  | Ohrbom et al. ....     | 526/312    |
| 6,403,709 B2      | 6/2002  | Ramesh et al. ....     | 525/95     |
| 6,462,139 B1      | 10/2002 | Das et al. ....        |            |
| 6,503,983 B1      | 1/2003  | Morrison et al. ....   | 524/804    |
| 6,506,836 B1      | 1/2003  | Bremser et al. ....    | 525/64     |
| 6,512,026 B1      | 1/2003  | Ott et al. ....        |            |
| 6,534,588 B1      | 3/2003  | Löcken et al. ....     | 524/591    |
| 6,566,476 B2      | 5/2003  | Ohrbom et al. ....     | 526/312    |
| 6,670,043 B2      | 12/2003 | Barkac et al. ....     |            |
| 2002/0035289 A1   | 3/2002  | Walter et al. ....     | 560/157    |
| 2002/0086966 A1   | 7/2002  | Weise et al. ....      | 526/312    |
| 2002/0103319 A1   | 8/2002  | Ohrbom et al. ....     | 526/312    |
| 2002/0132921 A1   | 9/2002  | Ramesh et al. ....     | 525/88     |
| 2003/0078337 A1 * | 4/2003  | Bremser et al. ....    | 524/502    |
| 2003/0091832 A1   | 5/2003  | Ohrbom et al. ....     | 428/423.1  |
| 2003/0100673 A1   | 5/2003  | Bendix et al. ....     | 524/801    |
| 2003/0143414 A1   | 7/2003  | Bendix et al. ....     | 428/500    |

## OTHER PUBLICATIONS

|                                                                             |
|-----------------------------------------------------------------------------|
| Rink, et al., 10/049,607, filed Feb. 14, 2002.                              |
| Nickolaus et al., 10/250,694, Jul. 3, 2003.                                 |
| Bendix et al., 10/148,428, May 29, 2002.                                    |
| Clauss, 10/148,295, filed May 29, 2002.                                     |
| Bremser, 10/018,703, filed Dec. 13, 2001.                                   |
| Bremser, 10/018,352, filed Dec. 7, 2001.                                    |
| Bremser, 10/018,351, filed Dec. 7, 2001.                                    |
| Bendix et al., 10/148,427, filed May 29, 2002.                              |
| Derwent Accession No. 1996-056019, English Abstract for JP07316242.         |
| Derwent Accession No. 1999-502399, English Abstract for JP11217409.         |
| Derwent Accession No. 1996-094214, English Abstract for JP08003208.         |
| Derwent Accession No. 1986-152526, English Abstract for NIPPON, JP61085417. |
| English Abstract for, Dalibor, DE 3546594, filed Dec. 10, 1987.             |
| English Abstract for Grutter, EP 358 221, filed Mar. 14, 1990.              |
| English Abstract for Knoll, et al., EP 732 359, filed Sep. 18, 1996.        |

\* cited by examiner

**COLORING AND/OR EFFECT-CREATING  
MULTILAYER ENAMEL COATING,  
METHOD FOR THE PRODUCTION  
THEREOF AND ITS USE**

This application is a National Phase Application of Patent Application PCT/EP00/05825 filed on Jun. 23, 2000.

The present invention relates to a novel multicoat color and/or effect coating system for a primed or an unprimed substrate. The present invention further relates to a novel process for producing a multicoat color and/or effect coating system on a primed or unprimed substrate. The present invention relates not least to the use of the novel multicoat and/or effect coating system, and of the novel process for producing it, in automotive OEM finishing and refinishing, in industrial coating, including container coating and coil coating, and in furniture coating.

Multicoat color and/or effect coating systems for primed or unprimed substrates are known. Normally, they comprise a surfacer coat, which absorbs mechanical energy, and a solid-color and/or effect topcoat. In another variant, they comprise a surfacer coat, a color and/or effect basecoat, and a clearcoat. For the coating of plastics, it is also common to employ a multicoat system which comprises a color and/or effect basecoat and a clearcoat. In many cases, such multicoat systems are produced by the wet-on-wet technique, in which in particular the basecoat film is merely dried but not cured before the application of the clearcoat film, and the basecoat film and clearcoat film are cured together.

In the coating materials used to produce known multicoat color and/or effect coating systems, constituents are frequently used that are prepared by free-radical polymerization of olefinically unsaturated monomers. These constituents are also referred to as binders. In the majority of cases, the binders of said type comprise acrylate copolymers.

Acrylate copolymers and coating materials comprising them are described, for example, in the patents EP-B-0 447 428, EP-B-0 593 454, EP-B-0 052 776, or DE-A-42 04 518.

Acrylate copolymers may be prepared by well-known polymerization processes in bulk, solution or emulsion. Polymerization techniques for preparing acrylate copolymers, especially polyacrylate resins, are general knowledge and are widely described (cf., e.g., Houben-Weyl, Methoden der organischen Chemie, 4th Edition, Volume 14/1, pages 24 to 255 (1961)).

Further examples of suitable copolymerization processes for preparing acrylate copolymers are described in patents DE-A-197 09 465, DE-C-197 09 476, DE-A-28 48 906, DE-A-195 24 182, EP-A-0 554 783, EP-B-0 650 979, WO 95/27742, DE-A-38 41 540, and WO 82/02387.

Suitable reactors for the copolymerization processes are the customary and known stirred vessels, cascades of stirred vessels, tube reactors, loop reactors, and Taylor reactors, as described for example in patents DE-B- 1071 241 and EP-A-0 498 583 or in the article by K. Kataoka in Chemical Engineering Science, Volume 50, No. 9, 1995, pages 1409 to 1416.

The free-radical polymerization used to prepare the acrylate copolymers is often very exothermic and difficult to control. The implications of this fact for the reaction regime are that it is necessary to avoid high monomer concentrations and/or the batch mode, where the entirety of the monomers is introduced as an initial charge in an aqueous medium, emulsified and subsequently polymerized to completion. Even the tailoring of defined molecular weights, molecular weight distributions, and other properties frequently causes difficulties. The tailoring of a certain profile

of properties in the acrylate copolymers, however, is of great importance for their use as binders in coating materials, since by this means it is possible to influence the profile of performance properties of the coating materials in a direct way.

There has therefore been no lack of attempts to control the free-radical copolymerization of olefinically unsaturated monomers in a targeted manner.

For instance, International Patent Application WO 98/01478 describes a process in which the copolymerization is conducted in the presence of a free-radical initiator and of a thiocarbonylthio compound as chain transfer agent.

International Patent Application WO 92/13903 describes a process for preparing copolymers having a low molecular weight by means of free-radical chain polymerization in the presence of a group transfer agent containing a carbon-sulfur double bond. These compounds act not only as chain transfer agents but also as growth regulators, so that only low molecular weight copolymers result.

International Patent Application WO 96/15157 discloses a process for preparing copolymers having a comparatively narrow molecular weight distribution, in which a monomer is reacted with a vinyl-terminated macromonomer in the presence of a free-radical initiator.

Furthermore, International Patent Application WO 98/37104 discloses the preparation of acrylate copolymers having defined molecular weights by means of free-radical polymerization in the presence of a chain transfer agent containing a C—C double bond and containing radicals which activate this double bond in terms of the free-radical addition reaction of monomers.

Despite the significant progress in this area, there is still a lack of a universally applicable process of controlled free-radical polymerization which in a simple manner provides chemically structured polymers, especially acrylate copolymers, and by means of which it is possible to tailor the profile of properties of the polymers in respect of their use in coating materials, which are used to produce multicoat color and/or effect coating systems.

As a result, it continues to be necessary to take other measures, in some cases more complex ones, to harmonize the profiles of properties and material compositions of the surfacers, basecoat materials and clearcoat materials in such a way that the multicoat color and/or effect coating systems have the high optical quality and intercoat adhesion required by the market and no longer give rise to problems such as deficient condensation resistance of the surfacer coats, cracking (mud cracking) in the basecoats, or leveling defects or surface structures in the clearcoats.

It is an object of the present invention to provide new multicoat color and/or effect coating systems and also new processes for producing them, in which at least one coat of the multicoat color and/or effect coating system is produced from a coating material which may be adapted in a simple manner to its respective use as surfacer, basecoat and/or clearcoat material. The aim is to realize this object in a simple manner by tailoring the profile of properties of the coating materials, in particular through the use of chemically structured polymers obtainable by means of controlled free-radical polymerization. The new multicoat color and/or effect coating systems which result should no longer have the disadvantages of the prior art but instead should exhibit outstanding optical quality, intercoat adhesion and condensation resistance and should not exhibit any cracking (mud cracking), leveling defects or surface structures. Moreover, it should be possible to use these chemically structured polymers as grinding resins which make it possible in an

advantageous manner to provide pigment pastes having a particularly good capacity for incorporation by mixing for the surfacers, basecoat and clearcoat materials used to produce the new multicoat color and/or effect coating systems.

Accordingly, we have found the novel multicoat color and/or effect coating system ML for a primed or unprimed substrate, which comprises, lying above one another in the stated sequence

- (1) a surfacer coat FL which absorbs mechanical energy, and 10
  - (2) a color and/or effect topcoat DL or
  - (1) a surfacer coat FL which absorbs mechanical energy,
  - (2) a color and/or effect basecoat BL, and
  - (3) a clearcoat KL or
  - (1) a color and/or effect basecoat BL and 15
  - (2) a clearcoat KL,
- wherein at least one coat FL and/or DL or BL and/or KL or FL, BL and/or KL, preferably at least two coats FL, BL and/or KL or all coats FL and DL or BL and KL or FL, BL and KL of the multicoat system ML has or have been produced from a coating material comprising at least one constituent (A) preparable by free-radical polymerization of
- a) at least one olefinically unsaturated monomer,
  - b) at least one olefinically unsaturated monomer different than the olefinically unsaturated monomer (a) and of the general formula I



in which the radicals R<sup>1</sup>, R<sup>2</sup>, R<sup>3</sup> and R<sup>4</sup> each independently of one another are hydrogen atoms or substituted or unsubstituted alkyl, cycloalkyl, alkylcycloalkyl, cycloalkylalkyl, aryl, alkylaryl, cycloalkylaryl, arylalkyl or arylcycloalkyl radicals, with the proviso that at least two of the variables R<sup>1</sup>, R<sup>2</sup>, R<sup>3</sup> and R<sup>4</sup> are substituted or unsubstituted aryl, arylalkyl or arylcycloalkyl radicals, especially substituted or unsubstituted aryl radicals;

in an aqueous medium.

In the text below, the novel multicoat color and/or effect coating system ML for a primed or unprimed substrate is referred to as the "multicoat system ML of the invention".

We have also found the novel process for producing a multicoat color and/or effect coating system ML on a primed or unprimed substrate by

- (I) preparing a surfacer film by applying a surfacer to the substrate,
  - (II) curing the surfacer film to give the surfacer coat FL,
  - (III) preparing a solid-color topcoat film by applying a solid-color coat material to the surfacer coat FL, and 45
  - (IV) curing the solid-color topcoat film to give the solid-color topcoat DL,
- or
- (I) preparing a basecoat film by applying a basecoat material to the substrate,
  - (II) drying the basecoat film,
  - (III) preparing a clearcoat film by applying a clearcoat material to the basecoat film, and 50
  - (IV) jointly curing the basecoat film and the clearcoat film to give the basecoat BL and the clearcoat KL,
- or
- (I) preparing a surfacer film by applying a surfacer to the substrate,
  - (II) curing the surfacer film to give the surfacer coat FL,
  - (III) preparing a basecoat film by applying a basecoat material to the surfacer coat FL, 65
  - (IV) drying the basecoat film,

- (V) preparing a clearcoat film by applying a clearcoat material to the basecoat film, and
- (VI) jointly curing the basecoat film and the clearcoat film to give the basecoat BL and the clearcoat KL, in which at least one of the coating materials employed in each case comprises at least one constituent (A) preparable by free-radical polymerization of
- a) at least one olefinically unsaturated monomer and
- b) at least one olefinically unsaturated monomer different than the olefinically unsaturated monomer (a) and of the general formula I



in which the radicals R<sup>1</sup>, R<sup>2</sup>, R<sup>3</sup> and R<sup>4</sup> each independently of one another are hydrogen atoms or substituted or unsubstituted alkyl, cycloalkyl, alkylcycloalkyl, cycloalkylalkyl, aryl, alkylaryl, cycloalkylaryl, arylalkyl or arylcycloalkyl radicals, with the proviso that at least two of the variables R<sup>1</sup>, R<sup>2</sup>, R<sup>3</sup> and R<sup>4</sup> are substituted or unsubstituted aryl, arylalkyl or arylcycloalkyl radicals, especially substituted or unsubstituted aryl radicals;

in an aqueous medium.

In the text below, the novel process for producing a multicoat color and/or effect coating system ML on a primed or unprimed substrate is referred to as the "process of the invention".

In the light of the prior art it was surprising that the complex object on which the present invention was based could be achieved by means of the process of the invention and the multicoat systems ML of the invention. A particular surprise was that the multicoat coating systems ML of the invention have outstanding optical quality, possess good intercoat adhesion and condensation resistance, and no longer exhibit cracking (mud cracking), leveling defects or surface structures. More surprising still was that the use of thixotropic agents or Theological assistance in basecoat materials used to produce perlescent effects and/or dichroic effects is substantially or, in some cases, entirely unnecessary.

In accordance with the invention, at least one coat of the multicoat system ML of the invention is produced from a coating material which comprises a constituent (A). It is of advantage in accordance with the invention if at least two coats, in particular all coats, of the multicoat system ML of the invention are produced from such coating materials.

In accordance with the invention, the constituent (A) is prepared by controlled free-radical polymerization of at least one olefinically unsaturated monomer (a) and at least one olefinically unsaturated monomer (b) which is different than the monomer (a).

Examples of suitable monomers (a) are

- a1) essentially acid-group-free (meth)acrylic esters such as (meth)acrylic alkyl or cycloalkyl esters having up to 20 carbon atoms in the alkyl radical, especially methyl, ethyl, propyl, n-butyl, sec-butyl, tert-butyl, hexyl, ethylhexyl, stearyl and lauryl acrylate or methacrylate; cycloaliphatic (meth)acrylic esters, especially cyclohexyl, isobornyl, dicyclopentadienyl, octahydro-4,7-methano-1H-indenemethanol or tert-butylcyclohexyl (meth)acrylate; (meth)acrylic oxaalkyl esters or oxacycloalkyl esters such as ethyltriglycol (meth)acrylate and methoxyoligoglycol (meth)acrylate having a molecular weight Mn of preferably 550, or other ethoxylated and/or propoxylated hydroxyl-free (meth)acrylic acid derivatives. These may contain minor amounts of (meth)acrylic alkyl or

cycloalkyl esters of higher functionality, such as the di(meth)acrylates of ethylene glycol, propylene glycol, diethylene glycol, dipropylene glycol, butylene glycol, 1,5-pentanediol, 1,6-hexanediol, octahydro-4,7-methano-1H-indenedimethanol or 1,2-, 1,3- or 1,4-cyclohexanediol; trimethylolpropane di- or tri(meth)acrylate; or pentaerythritol di-, tri- or tetra(meth)acrylate. For the purposes of the present invention, minor amounts of monomers of higher functionality in this case are to be understood as amounts which do not lead to crosslinking or gelling of the copolymers (A).

a2) Monomers which carry per molecule at least one hydroxyl group, amino group, alkoxyethylamino group or imino group and are essentially free from acid groups, such as hydroxyalkyl esters of acrylic acid, methacrylic acid or another alpha,beta-olefinically unsaturated carboxylic acid, which derive from an alkylene glycol esterified with the acid, or which are obtainable by reacting the alpha,beta-olefinically unsaturated carboxylic acid with an alkylene oxide, especially hydroxyalkyl esters of acrylic acid, methacrylic acid, ethacrylic acid, crotonic acid, maleic acid, fumaric acid or itaconic acid in which the hydroxyalkyl group contains up to 20 carbon atoms, such as 2-hydroxyethyl, 2-hydroxypropyl, 3-hydroxypropyl, 3-hydroxybutyl, 4-hydroxybutyl acrylate, methacrylate, ethacrylate, crotonate, maleate, fumarate or itaconate; or hydroxycycloalkyl esters such as 1,4-bis(hydroxymethyl)cyclohexane, octahydro-4,7-methano-1H-indenedimethanol or methylpropanediol monoacrylate, monomethacrylate, monoethacrylate, monocrotonate, monomaleate, monofumarate or monoitaconate; or reaction products of cyclic esters, such as epsilon-caprolactone, for example, and these hydroxy-alkyl or hydroxycycloalkyl esters; or olefinically unsaturated alcohols such as allyl alcohol or polyols such as trimethylolpropane monoallyl or diallyl ether or pentaerythritol monoallyl, diallyl or triallyl ether (as far as these monomers (a2) of higher functionality are concerned, the comments made above relating to the monomers (a1) of higher functionality apply analogously); N,N-dimethylaminoethyl acrylate, N,N-diethylaminoethyl methacrylate, allylamine or N-methyliminoethyl acrylate or N,N-di(methoxymethyl)aminoethyl acrylate and methacrylate or N,N-di(butoxymethyl)aminopropyl acrylate and methacrylate; monomers of this kind are used preferably to prepare self-crosslinking constituents (A).

a3) Monomers which carry per molecule at least one acid group which can be converted into the corresponding acid anion group, such as acrylic acid, methacrylic acid, ethacrylic acid, crotonic acid, maleic acid, fumaric acid or itaconic acid; olefinically unsaturated sulfonic or phosphonic acids or their partial esters; or mono(meth)acryloyloxyethyl maleate, succinate or phthalate.

a4) Vinyl esters of alpha-branched monocarboxylic acids having 5 to 18 carbon atoms in the molecule. The branched monocarboxylic acids can be obtained by reacting formic acid or carbon monoxide and water with olefins in the presence of a liquid, strongly acidic catalyst; the olefins may be cracking products of paraffinic hydrocarbons, such as mineral oil fractions, and may comprise both branched and straight-chain acyclic and/or cycloaliphatic olefins. The reaction of such olefins with formic acid or, respectively, with carbon monoxide and water produces a mixture of carboxylic acids in which the carboxyl groups are located predominantly on a quaternary carbon atom. Examples of other olefinic starting

materials are propylene trimer, propylene tetramer and diisobutylene. Alternatively, the vinyl esters (a4) may be prepared in a conventional manner from the acids, by reacting, for example, the acid with acetylene. Particular preference, owing to their ready availability, is given to using vinyl esters of saturated aliphatic monocarboxylic acids having 9 to 11 carbon atoms that are branched on the alpha carbon atom, but especially Versatic® acids.

- a5) Reaction products of acrylic acid and/or methacrylic acid with the glycidyl ester of an alpha-branched monocarboxylic acid having 5 to 18 carbon atoms per molecule, especially a Versatic® acid, or, instead of the reaction product, an equivalent amount of acrylic acid and/or methacrylic acid which is then reacted during or after the polymerization reaction with the glycidyl ester of an alpha-branched monocarboxylic acid having 5 to 18 carbon atoms per molecule, especially a Versatic® acid.
- a6) Cyclic and/or acyclic olefins such as ethylene, propylene, 1-butene, 1-pentene, 1-hexene, cyclohexene, cyclopentene, norbornene, butadiene, isoprene, cyclopentadiene and/or dicyclopentadiene.
- a7) (Meth)acrylamides such as (meth)acrylamide, N-methyl-, N,N-dimethyl-, N-ethyl-, N,N-diethyl-, N-propyl-, N,N-dipropyl-, N-butyl-, N,N-dibutyl-, N-cyclohexyl-, N,N-cyclohexylmethyl- and/or N-methylol-, N,N-dimethylol-, N-methoxymethyl-, N,N-di(methoxymethyl)-, N-ethoxymethyl- and/or N,N-di(ethoxyethyl)-(meth)acrylamide. Monomers of the last-mentioned kind are used in particular to prepare self-crosslinking constituents (A).
- a8) Monomers containing epoxide groups, such as the glycidyl esters of acrylic acid, methacrylic acid, ethacrylic acid, crotonic acid, maleic acid, fumaric acid and/or itaconic acid.
- a9) Vinylaromatic hydrocarbons such as styrene, alpha-alkylstyrenes, especially alpha-methylstyrene, and/or vinyltoluene; vinylbenzoic acid (all isomers), N,N-diethylaminostyrene (all isomers), alpha-methylvinylbenzoic acid (all isomers), N,N-diethylamino-alpha-methylstyrene (all isomers) and/or p-vinylbenzenesulfonic acid.
- a10) Nitriles such as acrylonitrile and/or methacrylonitrile.
- a11) Vinyl compounds, especially vinyl halides and/or vinylidene dihalides such as vinyl chloride, vinyl fluoride, vinylidene dichloride or vinylidene difluoride; N-vinylamides such as vinyl-N-methylformamide, N-vinylcaprolactam, 1-vinylimidazole or N-vinylpyrrolidone; vinyl ethers such as ethyl vinyl ether, n-propyl vinyl ether, isopropyl vinyl ether, n-butyl vinyl ether, isobutyl vinyl ether and/or vinyl cyclohexyl ether; and/or vinyl esters such as vinyl acetate, vinyl propionate, vinyl butyrate, vinyl pivalate and/or the vinyl ester of 2-methyl-2-ethylheptanoic acid.
- a12) Allyl compounds, especially allyl ethers and allyl esters such as allyl methyl, ethyl, propyl or butyl ether or allyl acetate, propionate or butyrate.
- a13) Polysiloxane macromonomers having a number-average molecular weight Mn of from 1000 to 40 000 and having on average from 0.5 to 2.5 ethylenically unsaturated double bonds per molecule; especially polysiloxane macromonomers having a number-average molecular weight Mn of from 2000 to 20 000, with particular preference from 2500 to 10 000 and, in particular, from 3000 to 7000 and having on average from 0.5 to 2.5, preferably from 0.5 to 1.5, ethylenically unsaturated double bonds per molecule, as are described in DE-A 38 07 571 A1 on pages 5 to 7, in DE-A 37 06 095 in columns

3 to 7, in EP-B 0 358 153 on pages 3 to 6, in U.S. Pat. No. A 4,754,014 in columns 5 to 9, in DE-A 44 21 823 or in International Patent Application WO 92/22615 on page 12 line 18 to page 18 line 10. and/or  
 a14) Acryloxy silane-containing vinyl monomers, preparable by reacting hydroxyl-functional silanes with epichlorohydrin and then reacting the reaction product with (meth) acrylic acid and/or with hydroxyalkyl and/or hydroxycycloalkyl esters of (meth)acrylic acid (cf. monomers a2).

Each of the abovementioned monomers (a1) to (a14) may be polymerized on their own with the monomers (b). In accordance with the invention, however, it is advantageous to use at least two monomers (a), since by this means it is possible to vary the profile of properties of the resulting constituents (A), i.e., copolymers (A), very widely, in a particularly advantageous manner, and to tailor said profile of properties specifically to the particular intended use of the coating material. In particular, it is possible in this way to incorporate into the copolymers (A) functional groups by means of which the copolymers (A) become hydrophilic, so that they may be dissolved or dispersed in aqueous media. It is also possible to incorporate functional groups (afg) capable of entering into thermal crosslinking reactions with the complementary functional groups (bfg), described below, of the crosslinking agents (B). It is also possible to incorporate functional groups which give the constituent (A) self-crosslinking properties, such as N-methylol groups or N-alkoxymethyl groups.

In accordance with the invention, very particular advantages result if the monomers (a) used comprise the monomers (a1) and (a2) and also, if desired, (a3).

In accordance with the invention, the monomers (b) used comprise compounds of the general formula I.

In the general formula I, the radicals R<sup>1</sup>, R<sup>2</sup>, R<sup>3</sup> and R<sup>4</sup> each independently of one another are hydrogen atoms or substituted or unsubstituted alkyl, cycloalkyl, alkylcycloalkyl, cycloalkylalkyl, aryl, alkylaryl, cycloalkylaryl, arylalkyl or arylcycloalkyl radicals, with the proviso that at least two of the variables R<sup>1</sup>, R<sup>2</sup>, R<sup>3</sup> and R<sup>4</sup> are substituted or unsubstituted aryl, arylalkyl or arylcycloalkyl radicals, especially substituted or unsubstituted aryl radicals.

Examples of suitable alkyl radicals are methyl, ethyl, propyl, isopropyl, n-butyl, isobutyl, tert-butyl, amyl, hexyl or 2-ethylhexyl.

Examples of suitable cycloalkyl radicals are cyclobutyl, cyclopentyl or cyclohexyl.

Examples of suitable alkylcycloalkyl radicals are methylenecyclohexane, ethylenecyclohexane or propane-1,3-diylcyclohexane.

Examples of suitable cycloalkylalkyl radicals are 2-,3- or 4-methyl-, -ethyl-, -propyl- or -butylcyclohex-1-yl.

Examples of suitable aryl radicals are phenyl, naphthyl or biphenyl, preferably phenyl and naphthyl, and especially phenyl.

Examples of suitable alkylaryl radicals are benzyl or ethylene- or propane-1,3-diylbenzene.

Examples of suitable cycloalkylaryl radicals are 2-, 3- or 4-phenylcyclohex-1-yl.

Examples of suitable arylalkyl radicals are 2-, 3- or 4-methyl-, -ethyl-, -propyl- or -butylphen-1-yl. Examples of suitable arylcycloalkyl radicals are 2-, 3- or 4-cyclohexylphen-1-yl.

The above-described radicals R<sup>1</sup>, R<sup>2</sup>, R<sup>3</sup> and R<sup>4</sup> may be substituted. The substituents used may comprise electron-withdrawing or electron-donating atoms or organic radicals.

Examples of suitable substituents are halogen atoms, especially chlorine and fluorine, nitrile groups, nitro groups,

partially or fully halogenated, especially chlorinated and/or fluorinated, alkyl, cycloalkyl, alkylcycloalkyl, cycloalkylalkyl, aryl, alkylaryl, cycloalkylaryl, arylalkyl and arylcycloalkyl radicals, including those exemplified above, especially tertbutyl; aryloxy, alkyloxy and cycloalkyloxy radicals, especially phenoxy, naphthoxy, methoxy, ethoxy, propoxy, butyloxy or cyclohexyloxy; arylthio, alkylthio and cycloalkylthio radicals, especially phenylthio, naphthylthio, methylthio, ethylthio, propylthio, butylthio or cyclohexylthio; hydroxyl groups; and/or primary, secondary and/or tertiary amino groups, especially amino, N-methylamino, N-ethylamino, N-propylamino, N-phenylamino, N-cyclohexylamino, N,N-dimethylamino, N,N-diethylamino, N,N-dipropylamino, N,N-diphenylamino, N,N-dicyclohexylamino, N-cyclohexyl-N-methylamino and N-ethyl-N-methylamino.

Examples of monomers (b) whose use is particularly preferred in accordance with the invention are diphenylethylene, dinaphthaleneethylene, cis- or trans-20 stilbene, vinylidenebis(4-N,N-dimethylamino-benzene), vinylidenebis(4-aminobenzene), and vinylidenebis(4-nitrobenzene).

In accordance with the invention, the monomers (b) may be used individually or as a mixture of at least two monomers (b).

In terms of the reaction regime and the properties of the resultant copolymers (A), especially the acrylate copolymers (A), diphenylethylene is of very particular advantage and is therefore used with very particular preference in accordance 30 with the invention.

The monomers (a) and (b) to be used in accordance with the invention are reacted with one another in the presence of at least one free-radical initiator to form the copolymer (A). Examples of initiators which can be used are: dialkyl 35 peroxides, such as di-tert-butyl peroxide or dicumyl peroxide; hydroperoxides, such as cumene hydroperoxide or tert-butyl hydroperoxide; peresters, such as tert-butyl perbenzoate, tert-butyl perpivalate, tert-butyl per-3,5,5-trimethylhexanoate or tert-butyl per-2-ethylhexanoate; potassium, sodium or ammonium peroxodisulfate; azodinitriles such as azobisisobutyronitrile; C-C-cleaving initiators such as benzpinacol silyl ethers; or a combination of a nonoxidizing initiator with hydrogen peroxide.

It is preferred to add comparatively large amounts of free-radical initiator, the proportion of the initiator in the reaction mixture being, based in each case on the overall amount of the monomers (a) and of the initiator, with particular preference from 0.5 to 50% by weight, with very particular preference from 1 to 20% by weight, and in particular from 2 to 15% by weight.

Preferably, the weight ratio of initiator to the monomers (b) is from 4:1 to 1:4, with particular preference from 3:1 to 1:3, and in particular from 2:1 to 1:2. Further advantages result if the initiator is used in excess within the stated limits.

The free-radical copolymerization is preferably conducted in the apparatus mentioned at the outset, especially stirred vessels or Taylor reactors, the Taylor reactors being designed such that the conditions of Taylor flow are met over the entire reactor length, even if the kinematic viscosity of the reaction medium alters greatly, and in particular increases, owing to the copolymerization.

In accordance with the invention, the copolymerization is conducted in an aqueous medium.

The aqueous medium comprises essentially water. The aqueous medium may here include minor amounts of the below-detailed crosslinking agents (B), reactive diluents (F), coatings additives (G) and/or organic solvents (H) and/or

other dissolved solid, liquid or gaseous organic and/or inorganic substances of low and/or high molecular mass, especially surface-active substances, provided these do not adversely affect, or even inhibit, the copolymerization. In the context of the present invention, a "minor amount" is to be understood as an amount which does not remove the aqueous character of the aqueous medium.

Alternatively, the aqueous medium may comprise straight water.

The copolymerization is preferably conducted in the presence of at least one base. Particular preference is given to low molecular mass bases such as sodium hydroxide solution, potassium hydroxide solution, ammonia, diethanolamine, triethanolamine, mono-, di- and triethylamine, and/or dimethylethanolamine, especially ammonia and/or di- and/or triethanolamine.

The copolymerization is advantageously conducted at temperatures above room temperature and below the lowest decomposition temperature of the monomers used in each case, preference being given to a chosen temperature range of from 10 to 150° C., with very particular preference from 70 to 120° C., and in particular from 80 to 110° C.

When using particularly volatile monomers (a) and/or (b), the copolymerization may also be conducted under pressure, preferably under from 1.5 to 3000 bar, with particular preference from 5 to 1500 bar, and in particular from 10 to 1000 bar.

In terms of the molecular weight distribution, there are no restrictions whatsoever imposed on the constituent (A). Advantageously, however, the copolymerization is conducted so as to give a molecular weight distribution  $M_w/M_n$ , measured by gel permeation chromatography using polystyrene as standard, of  $\leq 4$ , with particular preference  $\leq 2$ , and in particular  $\leq 1.5$ , and in certain cases even  $\leq 1.3$ . The molecular weights of the constituents (A) may be controlled within wide limits by the choice of ratio of monomer (a) to monomer (b) to free-radical initiator. In this context, the amount of monomer (b) in particular determines the molecular weight, specifically such that, the higher the proportion of monomer (b), the lower the resultant molecular weight.

The constituent (A) resulting from the copolymerization is obtained as a mixture with the aqueous medium, generally in the form of a dispersion. In this form it can be processed further directly or else used as a macroinitiator for further reaction with at least one further monomer (a) in a second stage (ii). The constituent (A) resulting in the first stage (i), however, may also be isolated as a solid and then reacted further.

The further reaction in accordance with the stage (ii) is preferably conducted under the standard conditions for a free-radical polymerization, it being possible for suitable solvents (H) and/or reactive diluents (F) to be present. 5 Stages (i) and (ii) in the context of the process of the invention may be conducted separately from one another, both spatially and temporally. In addition, however, stages (i) and (ii) may also be carried out in succession in one reactor. For this purpose, the monomer (b) is first reacted with at least one monomer (a), completely or partially depending on the desired application and the desired properties, after which at least one further monomer (a) is 10 added and the mixture is subjected to free-radical polymerization. In another embodiment, at least two monomers (a) are used from the start, the monomer (b) being first reacted with one of the at least two monomers (a) and then the resultant reaction product (A) being reacted, above a certain molecular weight, with the further monomer (a) as well.

15 20 Depending on the reaction regime, it is possible in accordance with the invention to prepare endgroup-functionalized polymers, block, multiblock and gradient copolymers, star polymers, graft copolymers, and branched copolymers as constituents (A).

25 30 The constituent (A) may include at least one, preferably at least two, functional groups (afg) which are able to enter into thermal crosslinking reactions with complementary functional groups (bfg) of the crosslinking agents (B) described below. The functional groups (afg) may be introduced into the constituent (A) by way of the monomers (a) or may be introduced following its synthesis, by means of 35 40 polymer-analogous reactions.

45 Examples of suitable complementary reactive functional groups (afg) and (bfg) which enter into crosslinking reactions, for use in accordance with the invention, are summarized in the following overview. In the overview, the variable  $R^5$  is a substituted or unsubstituted alkyl, cycloalkyl, alkylcycloalkyl, cycloalkylalkyl, aryl, alkylaryl, cycloalkylaryl, arylalkyl or arylcycloalkyl radicals; the variables  $R^6$  and  $R^7$  are identical or different alkyl, cycloalkyl, alkylcycloalkyl or cycloalkylalkyl radicals, or are linked with one another to form an aliphatic or heteroaliphatic ring. Examples of suitable radicals of this kind are those listed above in connection with the radicals  $R^1$ ,  $R^2$ ,  $R^3$  and  $R^4$ .

Overview: Examples of complementary functional groups (afg) and (bfg) in the

| constituent (A) and crosslinking agent (B)<br>or<br>crosslinking agent (B) and constituent (A) |                                                                                                           |
|------------------------------------------------------------------------------------------------|-----------------------------------------------------------------------------------------------------------|
| $-\text{SH}$                                                                                   | $-\text{C}(\text{O})-\text{OH}$                                                                           |
| $-\text{NH}_2$                                                                                 | $-\text{C}(\text{O})-\text{O}-\text{C}(\text{O})-$                                                        |
| $-\text{OH}$                                                                                   | $-\text{NCO}$                                                                                             |
| $-\text{O}-(\text{CO})-\text{NH}-(\text{CO})-\text{NH}_2$                                      | $-\text{NH}-\text{C}(\text{O})-\text{OR}^5$                                                               |
| $-\text{O}-(\text{CO})-\text{NH}_2$                                                            | $-\text{CH}_2-\text{OH}$                                                                                  |
|                                                                                                | $-\text{CH}_2-\text{O}-\text{CH}_3$                                                                       |
|                                                                                                | $-\text{NH}-\text{C}(\text{O})-\text{CH}(-\text{C}(\text{O})\text{OR}^5)_2$                               |
|                                                                                                | $-\text{NH}-\text{C}(\text{O})-\text{CH}(-\text{C}(\text{O})\text{OR}^5)(-\text{C}(\text{O})-\text{R}^5)$ |
|                                                                                                | $-\text{NH}-\text{C}(\text{O})-\text{NR}^6\text{R}^7$                                                     |
|                                                                                                | $=\text{Si}(\text{OR}^5)_2$                                                                               |
|                                                                                                |                      |

-continued

---

 constituent (A) and crosslinking agent (B)  
 or  
 crosslinking agent (B) and constituent (A)
 

---



15

The selection of the respective complementary groups (afg) and (bfg) is guided on the one hand by the consideration that, during storage, they should not enter into any unwanted reactions and/or should not disrupt or inhibit curing, if appropriate, with actinic radiation, and on the other hand by the temperature range within which thermal curing is to take place.

In this context, especially with regard to heat-sensitive substrates such as plastics, it is of advantage in accordance with the invention to choose a temperature range which does not exceed 100° C., and in particular does not exceed 80° C. In the light of these boundary conditions, complementary functional groups which have proven advantageous are hydroxyl groups and isocyanate groups, or carboxyl groups and epoxy groups, which are therefore employed with preference, in accordance with the invention, in the coating materials of the invention that are present as two-component or multi-component systems. Particular advantages result if the hydroxyl groups are used as functional groups (afg) and the isocyanate groups as functional groups (bfg).

If higher crosslinking temperatures, for example from 100° C. to 180° C., may be employed, which is preferred in accordance with the invention, suitable coating materials also include one-component systems, in which the functional groups (afg) are preferably thio, amino, hydroxyl, carbamate, allophanate, carboxyl and/or (meth)acrylate groups, but especially hydroxyl groups, and the functional groups (bfg) are preferably anhydride, carboxyl, epoxy, blocked isocyanate, urethane, methylol, methylol ether, siloxane, amino, hydroxyl and/or beta-hydroxyalkylamide groups.

The constituent (A) and, respectively, the coating material produced using it, however, may also film without a crosslinking agent (B) and still form an ideal coating. In this case, the constituent (A) is physically curing. In the context of the present invention, physical curing and curing by way of the above-described complementary groups (afg) and (bfg) are collected together under the term "thermal curing".

The proportion of the constituent (A) for use in accordance with the invention in the coating material may vary very widely and is also guided in particular by whether the coating material is to be used for the mechanical-energy-absorbing surfacer coat FL, the color and/or effect topcoat DL, the color and/or effect basecoat BL, or the clearcoats KL. Advantageously, the proportion is from 1 to 90, preferably from 2 to 80, with particular preference from 3 to 75, and in particular from 4 to 70% by weight, based in each case on the overall solids content of the coating material.

The coating material may further comprise at least one constituent (A') comprising a customary and known binder (A') with at least one functional group (afg). Examples of

suitable binders (A') are linear and/or branched and/or block, comb and/or random poly(meth)acrylates or acrylate copolymers, polyesters, alkyds, amino resins, polyurethanes, acrylated polyurethanes, acrylated polyesters, polylactones, polycarbonates, polyethers, epoxy resin-amine adducts, (meth)acrylate diols, partially hydrolyzed polyvinyl esters or polyureas, which contain said functional groups (afg). If used, their proportion in the coating material of the invention is preferably from 1 to 50, preferably from 2 to 40, with particular preference from 3 to 30, and in particular from 4 to 25% by weight, based in each case on the overall solids content of the coating material.

The coating material may further comprise at least one crosslinking agent (B) which contains at least two, especially three, of the complementary functional groups (bfg) described in detail above.

Where the coating material comprises a two-component or multicomponent system, polyisocyanates and/or polyepoxides, but especially polyisocyanates, are used as crosslinking agents (B).

Examples of suitable polyisocyanates (B) are organic polyisocyanates, especially so-called paint polyisocyanates, having free isocyanate groups attached to aliphatic, cycloaliphatic, araliphatic and/or aromatic moieties. Preference is given to polyisocyanates having from 2 to 5 isocyanate groups per molecule and viscosities of from 100 to 10 000, preferably from 100 to 5000, and in particular from 100 to 2000 mPa.s (at 23° C.). If desired, small amounts of organic solvent (H), preferably from 1 to 25% by weight based on straight polyisocyanate, may be added to the polyisocyanates in order to make it easier to incorporate the isocyanate and, if appropriate, to reduce the viscosity of the polyisocyanate to a level within the abovementioned ranges. Examples of suitable solvent additives to the polyisocyanates are ethoxyethyl propionate, amyl methyl ketone, and butyl acetate. Furthermore, the polyisocyanates (B) may have been hydrophilically or hydrophobically modified in a customary and known manner.

Examples of suitable polyisocyanates (B) are described, for example, in "Methoden der organischen Chemie", Houben-Weyl, Volume 14/2, 4th Edition, Georg Thieme Verlag, Stuttgart, 1963, pages 61 to 70, and by W. Siefken, Liebigs Annalen der Chemie, Volume 562, pages 75 to 136.

Further examples of suitable polyisocyanates (B) are polyisocyanates containing isocyanurate, biuret, allophanate, iminooxadiazinedione, urethane, urea and/or uretdione groups. Polyisocyanates containing urethane groups, for example, are prepared by reacting some of the isocyanate groups with polyols, such as trimethylolpropane and glycerol, for example. Preference is given to the use of aliphatic or cycloaliphatic polyisocyanates, especially hex-

amethylene diisocyanate, dimerized and trimerized hexamethylene diisocyanate, isophorone diisocyanate, 2-isocyanatopropylcyclohexyl isocyanate, dicyclohexylmethane 2,4'-diisocyanate, dicyclohexylmethane 4,4'-diisocyanate, or 1,3-bis(isocyanatomethyl)cyclohexane (BIC), diisocyanates derived from dimeric fatty acids, as marketed under the commercial designation DDI 1410 by Henkel, 1,8-diisocyanato-4-isocyanatomethyloctane, 1,7-diisocyanato-4-isocyanatomethylheptane or 1-iso-cyanato-2-(3-isocyanatopropyl)cyclohexane, or mixtures of these polyisocyanates.

Examples of suitable polyepoxides (B) are all known aliphatic and/or cycloaliphatic and/or aromatic polyepoxides, examples being those based on bisphenol A or bisphenol F. Other suitable examples of polyepoxides are the polyepoxides available commercially under the designations Epikote® from Shell, Denacol® from Nagase Chemicals Ltd., Japan, such as Denacol EX-411 (pentaerythritol polyglycidyl ether), Denacol EX-321 (trimethylolpropane polyglycidyl ether), Denacol EX-512 (polyglycerol polyglycidyl ether), and Denacol EX-521 (polyglycerol polyglycidyl ether).

In the case of the one-component systems, the crosslinking agents (B) used react at relatively high temperatures with the functional groups of the binders to build up a three-dimensional network. Of course, such crosslinking agents (B) may be used as well in the multicomponent systems, in minor amounts. In the context of the present invention, a "minor amount" is a proportion which does not disrupt, let alone prevent, the principal crosslinking reaction.

Examples of suitable crosslinking agents (B) of this kind are blocked polyisocyanates. Examples of suitable polyisocyanates for preparing the blocked polyisocyanates are those described above.

Examples of suitable blocking agents are the blocking agents known from U.S. Pat. No. 4,444,954, such as

- i) phenols such as phenol, cresol, xylenol, nitrophenol, chlorophenol, ethylphenol, t-butylphenol, hydroxybenzoic acid, esters of this acid, or 2,5-di-tert-butyl-4-hydroxytoluene;
- ii) lactams, such as  $\epsilon$ -caprolactam,  $\delta$ -valerolactam,  $\gamma$ -butyrolactam or  $\beta$ -propiolactam;
- iii) active methylenic compounds, such as diethyl malonate, dimethyl malonate, ethyl or methyl acetoacetate, or acetylacetone;
- iv) alcohols such as methanol, ethanol, n-propanol, isopropanol, n-butanol, isobutanol, t-butanol, n-amyl alcohol, t-amyl alcohol, lauryl alcohol, ethylene glycol monomethyl ether, ethylene glycol monoethyl ether, ethylene glycol monobutyl ether, diethylene glycol monomethyl ether, diethylene glycol monoethyl ether, propylene glycol monomethyl ether, methoxymethanol, glycolic acid, glycolic esters, lactic acid, lactic esters, methylolurea, methylolmelamine, diacetone alcohol, ethylenechlorohydrin, ethylenebromohydrin, 1,3-dichloro-2-propanol, 1,4-cyclohexyldimethanol or aceto-cyanohydrin;
- v) mercaptans such as butyl mercaptan, hexyl mercaptan, t-butyl mercaptan, t-dodecyl mercaptan, 2-mercaptopbenzothiazole, thiophenol, methylthio-phenol or ethylthiophenol;
- vi) acid amides such as acetoanilide, acetoanisidinamide, acrylamide, methacrylamide, acetamide, stearamide or benzamide;
- vii) imides such as succinimide, phthalimide or maleimide;
- viii) amines such as diphenylamine, phenylnaphthylamine, xylidine, N-phenylxylidine, carbazole, aniline, naphthylamine, butylamine, dibutylamine or butylphenylamine;

- ix) imidazoles such as imidazole or 2-ethylimidazole;
- x) ureas such as urea, thiourea, ethyleneurea, ethylenethiourea or 1,3-diphenylurea;
- xi) carbamates such as phenyl N-phenylcarbamate or 2-oxazolidone;
- xii) imines such as ethyleneimine;
- xiii) oximes such as acetone oxime, formaldoxime, acetaldoxime, acetoxime, methyl ethyl ketoxime, diisobutyl ketoxime, diacetyl monoxime, benzophenone oxime or chlorohexanone oximes;
- xiv) salts of sulfurous acid such as sodium bisulfite or potassium bisulfite;
- xv) hydroxamic esters such as benzyl methacrylohydroxamate (BMH) or allyl methacrylohydroxamate; or
- xvi) substituted pyrazoles, imidazoles or triazoles; and also mixtures of these blocking agents, especially dimethylpyrazole and triazoles, malonic esters and acetocrylic esters or dimethylpyrazole and succinimide.

As crosslinking agents (B) it is also possible to use tris(alkoxycarbonylamino)triazines (TACIs) of the general formula



Examples of suitable tris(alkoxycarbonylamino)triazines (B) are described in U.S. Pat. No. 4,939,213, U.S. Pat. No. 5,084,541, and EP-A-0 624 577. Use is made in particular of the tris(methoxy-, tris(butoxy- and/or tris(2-ethylhexoxycarbonylamino)triazines.

The methyl butyl mixed esters, the butyl 2-ethylhexyl mixed esters, and the butyl esters are of advantage. They have the advantage over the straight methyl ester of better solubility in polymer melts, and also have less of a tendency to crystallize out.

Especiably suitable crosslinking agents (B) are amino resins, examples being melamine resins, guanamine resins, and urea resins. Any amino resin suitable for transparent topcoats or clearcoats, or a mixture of such amino resins, may be used here. For further details, reference is made to Römpf Lexikon "Lacke und Druckfarben", Georg Thieme Verlag, 1998, page 29, "Amino resins", and the textbook "Lackadditive" [Additives for Coatings] by Johan Bieleman, Wiley-VCH, Weinheim, New York, 1998, pages 242 ff., or the book "Paints, Coatings and Solvents", second, completely revised edition, D. Stoye and W. Freitag (eds.), Wiley-VCH, Weinheim, New York, 1998, pages 80 ff. Also suitable are the customary and known amino resins some of whose methylol and/or methoxymethyl groups have been defunctionalized by means of carbamate or aliphonate groups. Crosslinking agents of this kind are described in U.S. Pat. No. 4,710,542 and EP-B-0 245 700 and also in the article by B. Singh and coworkers, "Carbamylmethylated Melamines, Novel Crosslinkers for the Coatings Industry" in Advanced Organic Coatings Science and Technology Series, 1991, Volume 13, pages 193 to 207.

Further examples of suitable crosslinking agents (B) are beta-hydroxyalkylamides such as N,N,N',N'-tetrakis(2-hydroxyethyl)adipamide or N,N,N',N'-tetrakis(2-hydroxypropyl)adipamide.

## 15

Further examples of suitable crosslinking agents (B) are siloxanes, especially siloxanes containing at least one trialkoxysilane or dialkoxysilane group.

Further examples of suitable crosslinking agents (B) are polyanhydrides, especially polysuccinic anhydride.

Further examples of suitable crosslinking agents (B) are compounds containing on average at least two groups amenable to transesterification, examples being reaction products of malonic diesters and polyisocyanates or reaction products of monoisocyanates with esters and partial esters of malonic acid with polyhydric alcohols, as described in European Patent EP-A-0 596 460.

The amount of the crosslinking agents (B) in the coating material may vary widely and is guided in particular, firstly, by the functionality of the crosslinking agents (B) and, secondly, by the number of crosslinking functional groups (afg) which are present in the binder (A), and also by the target crosslinking density. The skilled worker is therefore able to determine the amount of the crosslinking agents (B) on the basis of his or her general knowledge in the art, possibly with the aid of simple rangefinding experiments. Advantageously, the crosslinking agent (B) is present in the coating material of the invention in an amount of from 1 to 60, preferably from 2 to 50, and in particular from 3 to 45% by weight, based in each case on the overall solids content of the coating material of the invention. It is further advisable here to choose the amounts of crosslinking agent (B) and binder (A) such that in the coating material the ratio of functional groups (bfg) in the crosslinking agent (B) to functional groups (afg) in the binder (A) is from 2:1 to 1:2, preferably from 1.5:1 to 1:1.5, with particular preference from 1.2:1 to 1:1.2, and in particular from 1.1:1 to 1:1.1.

If the coating material is to be curable not only thermally but also with actinic radiation, especially UV radiation and/or electron beams (dual cure), it comprises at least one constituent (C) which is curable with actinic radiation. If, however, the coating material is to be curable predominantly (dual cure) or exclusively with actinic radiation, a circumstance which in the context of the process of the invention is particularly relevant to clearcoat materials, it must comprise a constituent (C).

Suitable constituents (C) are in principle all oligomeric and polymeric compounds that are curable with actinic radiation, especially UV radiation and/or electron beams, said compounds being commonly used in the field of UV curable or electron beam curable coating materials.

Radiation curable binders are used advantageously as constituents (C). Examples of suitable radiation curable binders (C) are (meth)acrylic-functional (meth)acrylic copolymers, polyether acrylates, polyester acrylates, unsaturated polyesters, epoxy acrylates, urethane acrylates, amino acrylates, melamine acrylates, silicone acrylates, isocyanato acrylates, and the corresponding methacrylates. It is preferred to use binders (C) that are free from aromatic structural units. Preference is therefore given to the use of urethane (meth)acrylates and/or polyester (meth)acrylates, with particular preference going to aliphatic urethane acrylates.

Where constituents (C) are used, they are present in the coating material in an amount of preferably from 1 to 80, more preferably from 1.5 to 70, with particular preference from 2 to 65, and in particular from 2.5 to 60% by weight, based in each case on the overall solids content of the coating material.

The coating material may further comprise at least one photoinitiator (D). If the coating material or the coats produced from it is/are to be crosslinked additionally (dual

## 16

cure) or exclusively with UV radiation in the context of the process of the invention, it is generally necessary to use a photoinitiator (D). Where used, it is present in the coating material of the invention in fractions of preferably from 0.01 to 10, more preferably from 0.1 to 8, and in particular from 0.5 to 6% by weight, based in each case on the overall solids content of the coating material of the invention.

Examples of suitable photoinitiators (D) are those of the Norrish II type, whose mechanism of action is based on an intramolecular variant of the hydrogen abstraction reactions as occur diversely in photochemical reactions (reference may be made here, by way of example, to Römpf Chemie Lexikon, 9th, expanded and revised edition, Georg Thieme Verlag, Stuttgart, Vol. 4, 1991) or cationic photoinitiators (reference may be made here, by way of example, to Römpf Lexikon "Lacke und Druckfarben", Georg Thieme Verlag, Stuttgart, 1998, pages 444 to 446), especially benzophenones, benzoins or benzoin ethers, or phosphine oxides. It is also possible to use, for example, the products available commercially under the names Irgacure® 184, Irgacure® 1800 and Irgacure® 500 from Ciba Geigy, Grenacure® MBF from Rahn, and Lucirin® TPO from BASF AG.

In addition to the photoinitiators (D), use may be made of customary sensitizers (D) such as anthracene in effective amounts.

Furthermore, the coating material may comprise at least one thermal crosslinking initiator (E). At from 80 to 120° C., these initiators form free radicals which start the crosslinking reaction. Examples of thermally labile free-radical initiators are organic peroxides, organic azo compounds or C-C-cleaving initiators such as dialkyl peroxides, peroxy-carboxylic acids, peroxydi-carbonates, peroxide esters, hydroperoxides, ketone peroxides, azo dinitriles, or benzpinacol silyl ethers. Particular preference is given to C-C-cleaving initiators, since their thermal cleavage does not produce any gaseous decomposition products which might lead to defects in the coating film. Where used, their amounts are generally from 0.01 to 10, preferably from 0.05 to 8, and in particular from 0.1 to 5% by weight, based in each case on the overall solids content of the coating material of the invention.

Moreover, the coating material may comprise at least one reactive diluent (F) curable thermally and/or with actinic radiation.

Examples of suitable thermally crosslinkable reactive diluents (F) are branched, cyclic and/or acyclic C<sub>9</sub>-C<sub>16</sub> alkanes functionalized with at least two hydroxyl groups, preferably dialkyloctanediols, especially the positionally isomeric diethyloctanediols.

Further examples of suitable thermally crosslinkable reactive diluents (F) are oligomeric polyols obtainable from oligomeric intermediates themselves obtained by metathesis reactions of acyclic monoolefins with cyclic monoolefins, by hydroformylation and subsequent hydrogenation; examples of suitable cyclic monoolefins are cyclobutene, cyclopentene, cyclohexene, cyclooctene, cycloheptene, norbornene or 7-oxanorbornene; examples of suitable acyclic monoolefins are present in hydrocarbon mixtures obtained in petroleum processing by cracking (C<sub>s</sub> cut); examples of suitable oligomeric polyols for use in accordance with the invention have a hydroxyl number (OHN) of from 200 to 450, a number-average molecular weight Mn of from 400 to 1000, and a mass-average molecular weight Mw of from 600 to 1100.

Further examples of suitable thermally crosslinkable reactive diluents (F) are hyperbranched compounds containing a tetrafunctional central group, derived from

17

dtrimethylolpropane, diglycerol, dtrimethylethane, pentaerythritol, tetrakis(2-hydroxyethyl)-methane, tetrakis(3-hydroxypropyl)methane or 2,2-bis-hydroxymethyl-1,4-butanediol (homopentaerythritol). These reactive diluents may be prepared in accordance with the customary and known methods of preparing hyperbranched and dendrimeric compounds. Suitable synthesis methods are described, for example, in patents WO 93/17060 or WO 96/12754 or in the book by G. R. Newkome, C. N. Moorefield and F. V. öggle, "Dendritic Molecules, Concepts, Syntheses, Perspectives", VCH, Weinheim, New York, 1996.

Further examples of suitable reactive diluents (F) are polycarbonate diols, polyester polyols, poly(meth)acrylate diols, and hydroxyl-containing polyadducts.

Examples of suitable reactive solvents which may be used as reactive diluents (F) are butyl glycol, 2-methoxypropanol, n-butanol, methoxybutanol, n-propanol, ethylene glycol monomethyl ether, ethylene glycol monoethyl ether, ethylene glycol monobutyl ether, diethylene glycol monomethyl ether, diethylene glycol monoethyl ether, diethylene glycol diethyl ether, diethylene glycol monobutyl ether, trimethylolpropane, ethyl 2-hydroxypropionate and 3-methyl-3-methoxybutanol, and also derivatives based on propylene glycol, e.g., isopropoxypropanol.

Examples of reactive diluents (F) used that may be crosslinked with actinic radiation are polysiloxane macromonomers, (meth)acrylic acid and other esters thereof, maleic acid and its esters, including monoesters, vinyl acetate, vinyl ethers, vinylureas, and the like. Examples that may be mentioned include alkylene glycol di(meth)acrylate, polyethylene glycol di(meth)acrylate, 1,3-butanediol di(meth)acrylate, vinyl (meth)acrylate, allyl (meth)acrylate, glycerol tri(meth)acrylate, trimethylolpropane tri(meth)acrylate, trimethylolpropane di(meth)acrylate, tripropylene glycol diacrylate, styrene, vinyltoluene, divinylbenzene, pentaerythritol tri(meth)acrylate, pentaerythritol tetra(meth)acrylate, dipropylene glycol di(meth)acrylate, hexanediol di(meth)acrylate, ethoxyethoxyethyl acrylate, N-vinylpyrrolidone, phenoxyethyl acrylate, dimethylaminoethyl acrylate, hydroxyethyl (meth)acrylate, butoxyethyl acrylate, isobornyl (meth)acrylate, dimethylacrylamide, and dicyclopentyl acrylate, and also the long-chain linear diacrylates described in EP-A-0 250 631 and having a molecular weight of from 400 to 4000, preferably from 600 to 2500. The acrylate groups may also, for example, be separated by a polyoxybutylene structure. Further candidates for use are 1,12-dodecyl diacrylate and the reaction product of 2 mol of acrylic acid with one mole of a dimeric fatty alcohol having generally 36 carbon atoms. Mixtures of the abovementioned monomers are also suitable.

Preferred for use as reactive diluents (F) are mono- and/or diacrylates, such as isobornyl acrylate, hexanediol diacrylate, tripropylene glycol diacrylate, Laromer® 8887 from BASF AG, and Actilane® 423 from Akros Chemicals Ltd., GB. Particular preference is given to the use of isobornyl acrylate, hexanediol diacrylate, and tripropylene glycol diacrylate.

Where used, the reactive diluents (F) are employed in an amount of preferably from 1 to 70, with particular preference from 2 to 65, and in particular from 3 to 50% by weight, based in each case on the overall solids content of the coating material of the invention.

The coating material of the invention may comprise customary coatings additives (G) in effective amounts. The nature and amount of the additives (G) are guided especially by the intended use of the coating material of the invention.

18

Advantageously, the additives (G) are not volatile under the processing and application conditions of the coating material of the invention.

Where the coating material is used as a surfacer FL, solid-color topcoat material DL and/or basecoat material BL, it mandatorily includes as coatings additives (G) at least one filler and/or at least one color and/or effect pigment (G) in customary and known, effective amounts. Preferably, the coating material comprises the fillers and/or pigments (G) in amounts of from 1 up to 95% by weight, with particular preference from 2 to 90% by weight, and in particular from 3 to 85% by weight, based in each case on the overall solids content of the coating material.

The pigments (G) may comprise organic or inorganic compounds and may impart color and/or effect. Owing to this large number of suitable pigments (G), therefore, the coating material of the invention ensures a universal breadth of use of the coating materials and permits the realization of a large number of shades and optical effects.

As effect pigments (G) it is possible to use metal flake pigments such as commercial aluminum bronzes, aluminum bronzes chromated in accordance with DE-A-36 36 183, and commercial stainless steel bronzes, and also nonmetallic effect pigments, such as perlescent pigments and/or interference pigments, for example. Examples of suitable inorganic color pigments (G) are titanium dioxide, iron oxides, Sicotrans yellow and carbon black. Examples of suitable organic color pigments (G) are indanthrene blue, Cromophthal red, Irgazine orange and Heliogen green.

Moreover the coating material, especially the surfacer FL, may comprise organic and inorganic fillers (G) in customary and known, effective amounts. Examples of suitable fillers are chalk, calcium sulfate, barium sulfate, silicates such as talc or kaolin, silicas, oxides such as aluminum hydroxide or magnesium hydroxide, or organic fillers such as textile fibers, cellulose fibers, polyethylene fibers, or wood flour. For further details, reference is made to Römpf Lexikon "Lacke und Druckfarben", Georg Thieme Verlag, 1998, pages 250 ff., "Fillers".

These additives (G) may also be incorporated into the coating materials by way of pigment pastes, with suitable grinding resins being, in particular, the above-described constituents (A) and also, if appropriate, the above-described constituents (A').

These additives (G) are omitted if the coating materials are used, in the context of the process of the invention, as clearcoat materials KL.

Examples of suitable additives (G) which may be present both in the clearcoat materials KL and in the surfacers FL, solid-color topcoat materials DL and basecoat materials BL of the invention are

UV absorbers;  
light stabilizers such as HALS compounds, benzoltriazoles or oxalanilides;  
free-radical scavengers;  
crosslinking catalysts such as dibutyltin dilaurate or lithium decanoate;  
slip additives;  
polymerization inhibitors;  
defoamers;  
neutralizing agents such as ammonia or dimethylethanolamine;  
emulsifiers, especially nonionic emulsifiers such as alkoxylated alkanols and polyols, phenols and alkylphenols or anionic emulsifiers such as alkali metal salts or ammonium salts of alkanecarboxylic acids,

19

alkanesulfonic acids, and sulfo acids of alkoxylated alkanols and polyols, phenols and alkylphenols; wetting agents such as siloxanes, fluorine compounds, carboxylic monoesters, phosphoric esters, polyacrylic acids and their copolymers, or polyurethanes; adhesion promoters such as tricyclodecanedimethanol; leveling agents; film-forming auxiliaries such as cellulose derivatives; transparent fillers based on silica, alumina or zirconium oxide; for further details reference is made to Römpf Lexikon "Lacke und Druckfarben", Georg Thieme Verlag, Stuttgart, 1998, pages 250 to 252; sag control agents such as ureas, modified ureas and/or silicas, as described for example in the references EP-A-192 304, DE-A-23 59 923, DE-A-18 05 693, WO 94/22968, DE-C-27 51 761, WO 97/12945 or "farbe+lack", 11/1992, pages 829 ff.; rheology control additives such as those known from patents WO 94/22968, EP-A-0 276 501, EP-A-0 249 201 or WO 97/12945; crosslinked polymeric microparticles, such as disclosed, for example, in EP-A-0 008 127; inorganic phyllosilicates such as aluminum-magnesium silicates, sodium-magnesium and sodium-magnesium-fluorine-lithium phyllosilicates of the montmorillonite type; silicas such as Aerosils; or synthetic polymers containing ionic and/or associative groups such as polyvinyl alcohol, poly(meth)acrylamide, poly(meth)acrylic acid, polyvinylpyrrolidone, styrene-maleic anhydride or ethylene-maleic anhydride copolymers and their derivatives, or hydrophobically modified ethoxylated urethanes or polyacrylates; flame retardants; and/or flattening agents.

Further examples of suitable coatings additives (G) of this kind are described in the textbook "Lackadditive" by Johan Bieleman, Wiley-VCH, Weinheim, New York, 1998.

The essential factor is that the above-described coatings additives (G), which may be present both in the surfacers, solid-color topcoats and basecoats and in the clearcoats, do not adversely affect the transparency and clarity of the coating material when it is used as clearcoat KL.

The coating material preferably comprises these coatings additives (G), which may be present both in the surfacers, solid-color topcoat materials and basecoat materials and in the clearcoat materials, in amounts of up to 40, with particular preference up to 30, and in particular up to 20% by weight, based in each case on the overall solids content of the coating material.

Not least, the coating materials of the invention, especially in the case of nonaqueous coating materials, may comprise from 1 to 70, preferably from 2 to 60% by weight (based on the application-ready coating material), of water-miscible and water-immiscible organic solvents (H), such as aliphatic, aromatic and/or cycloaliphatic hydrocarbons such as toluene or methylcyclohexane or decalin; alkyl esters of acetic acid or propionic acid; alkanols such as ethanol; ketones such as methyl isobutyl ketone; glycol ethers; glycol ether esters, and/or ethers such as tetrahydrofuran. In the context of the present invention it is also possible to use carbon dioxide as solvent (H).

The coating material of the invention may be present in different forms.

Thus, given an appropriate choice of its above-described constituents (A) and, if appropriate, of at least one of its constituents (A'), (B), (C), (D), (E), (F) and/or (G), it may be

20

present in the form of a liquid coating material which is essentially free from organic solvents and/or water (100% system).

However, the coating material may also comprise a solution or dispersion of the above-described constituents in organic solvents (H) and/or water. It is a further advantage of the coating material of the invention that in this case it is possible to establish solids contents of up to more than 80% by weight, based on the coating material.

10 Moreover, given an appropriate choice of its above-described constituents, the coating material of the invention may be a powder coating material. For this purpose, the constituent (B) may have been microencapsulated if it is a polyisocyanate. This powder coating material may then, if desired, be dispersed in water, to give a powder slurry coating material.

15 The coating material may be a two-component or multi-component system in which at least constituent (B) is stored separately from the other constituents and is not added to them until shortly before use. In this case, the coating material of the invention may also be aqueous, the constituent (B) preferably being present in a component comprising a solvent (H).

20 Furthermore, the coating material of the invention may be 25 part of a so-called mixer system or modular system, as described, for example, in patent DE-A-41 10 520, EP-A-0 608 773, EP-A-0 614 951, or EP-A-0 471 972.

25 Preferably, the coating material of the invention is in the form of an aqueous solution, a dispersion and/or an 30 emulsion, in particular a dispersion, since in this case there is no need to isolate the constituent (A) for use in accordance with the invention.

35 The preparation of the coating material from its constituents (A) and also, if appropriate, at least one of its constituents (A'), (B), (C), (D), (E), (F), (G) and/or (H) has no special features but instead takes place in a customary and known manner by mixing the constituents in appropriate mixing equipment such as stirred vessels, dissolvers or 40 extruders in accordance with the techniques suitable for the preparation of the respective coating materials.

The coating material of the invention is used to produce the multicoat systems ML of the invention on primed or unprimed substrates.

45 Suitable coating substrates are fundamentally all surfaces which are undamaged by curing of the coatings present thereon using heat and, if appropriate, actinic radiation; examples are metals, plastics, wood, ceramic, stone, textile, fiber composites, leather, glass, glass fibers, glass wool, rock wool, mineral-and resin-bound building materials, such as 50 plasterboard and cement slabs or roof tiles, and also assemblies of these materials. Accordingly, the multicoat system of the invention is fundamentally also suitable for applications outside of automotive finishing, in particular for furniture coating and industrial coating, including coil coating 55 and container coating. In the context of industrial coatings it is suitable for coating virtually all parts and articles for private or industrial use, such as radiators, domestic appliances, small metal parts, hubcaps or wheel rims.

In the case of electrically conductive substrates it is 60 possible to use primers which are produced in a customary and known manner from electrodeposition coating materials. For this purpose, both anodic and cathodic electrodeposition coating materials are suitable, but especially cathodic materials.

65 Using the multicoat system ML of the invention it is also possible in particular to coat primed or unprimed plastics such as, for example, ABS, AMMA, ASA, CA, CAB, EP,

## 21

UF, CF, MF, MPF, PF, PAN, PA, PE, HDPE, LDPE, LLDPE, UHMWPE, PET, PMMA, PP, PS, SB, PUR, PVC, RF, SAN, PBT, PPE, POM, PUR-RIM, SMC, BMC, PP-EPDM, and UP (abbreviated codes in accordance with DIN 7728T1). The plastics to be coated may of course also be polymer blends, modified plastics, or fiber reinforced plastics. It is also possible to employ the plastics commonly used in vehicle construction, especially motor vehicle construction.

Unfunctionalized and/or nonpolar substrate surfaces may be subjected prior to coating in a known manner to a pretreatment, such as with a plasma or by flaming, or may be provided with a water-based primer.

The multicoat systems ML of the invention may be produced in a variety of ways in accordance with the process of the invention.

In a first preferred variant, the process of the invention comprises the following steps:

- (I) preparing a surfacer film by applying a surfacer to the substrate,
- (II) curing the surfacer film to give the surfacer coat FL,
- (III) preparing a solid-color topcoat film by applying a solid-color topcoat material to the surfacer coat FL, and
- (IV) curing the solid-color topcoat film to give the solid-color topcoat DL.

In another preferred variant, the process of the invention comprises the following steps:

- (I) preparing a basecoat film by applying a basecoat material to the substrate,
- (II) drying the basecoat film,
- (III) preparing a clearcoat film by applying a clearcoat material to the basecoat film, and
- (IV) jointly curing the basecoat film and the clearcoat film to give the basecoat BL and the clearcoat KL (wet-on-wet technique).

A third preferred variant of the process of the invention comprises the steps of:

- (I) preparing a surfacer film by applying a surfacer to the substrate,
- (II) curing the surfacer film to give the surfacer coat FL,
- (III) preparing a basecoat film by applying a basecoat material to the surfacer coat FL,
- (IV) drying the basecoat film,
- (V) preparing a clearcoat film by applying a clearcoat material to the basecoat film, and
- (VI) jointly curing the basecoat film and the clearcoat film to give the basecoat BL and the clearcoat KL (wet-on-wet technique).

Which of the preferred variants is chosen depends on the intended use of the multicoat systems ML of the invention. For instance, the third variant, in particular, is employed with great preference in the context of automotive OEM finishing.

Accordingly, the multicoat systems ML of the invention may differ in their structure.

In a first preferred variant of the multicoat system ML of the invention,

- (1) a surfacer coat FL which absorbs mechanical energy, and
- (2) a color and/or effect topcoat DL

lie above one another in the stated sequence.

In a second preferred variant of the multicoat system ML of the invention,

- (1) a surfacer coat FL which absorbs mechanical energy,
- (2) a color and/or effect basecoat BL, and
- (3) a clearcoat KL

lie above one another in the stated sequence.

In a third preferred variant of the multicoat system ML of the invention,

- (1) a color and/or effect basecoat BL and
- (2) a clearcoat KL

lie above one another in the stated sequence. The third preferred variant is employed in particular in the context of coating plastics.  $\mu\text{m}$  [sic]

The application of the coating material in the context of the process of the invention may take place by any customary application method, such as spraying, knife coating, brushing, flow coating, dipping, or rolling. It is preferred to employ spray application methods, such as compressed air spraying, airless spraying, high-speed rotation, electrostatic spray application (ESTA), for example, alone or in conjunction with hot spray application such as hot air spraying, for example. Application may take place at temperatures of max. 70 to 80° C., so that appropriate application viscosities are attained without any change or damage to the coating material and its overspray (which may be intended for reprocessing) during the short period of thermal stress. For instance, hot spraying may be configured in such a way that the coating material is heated only very briefly in the spray nozzle or shortly before the spray nozzle.

The spray booth used for application may, for example, be operated with a circulation system, which may be temperature-controllable, and which is operated with an appropriate absorption medium for the overspray, an example of such medium being the coating material itself.

Where the coating material includes constituents (C) crosslinkable with actinic radiation, application is made under illumination with visible light with a wavelength of above 550 nm, or in the absence of light. By this means, material alteration or damage to the coating material and to the overspray is avoided.

The application methods described above may be used to produce all coats FL, DL, BL and KL and also, if desired, further coats.

In the process of the invention, the surfacer film, topcoat film, basecoat film and clearcoat film are applied in a wet film thickness such that their curing results in coats FL, DL, BL and KL having the thicknesses which are advantageous and necessary for their functions. In the case of the surfacer film FL, this thickness is from 10 to 150, preferably from 15 to 120, with particular preference from 20 to 100, and in particular from 25 to 90  $\mu\text{m}$ ; in the case of the topcoat DL it is from 5 to 90, preferably from 10 to 80, with particular preference from 15 to 60, and in particular from 20 to 50  $\mu\text{m}$ ; in the case of the basecoat BL it is from 5 to 50, preferably from 10 to 40, with particular preference from 12 to 30 and in particular from 15 to 25  $\mu\text{m}$ , and in the case of the clearcoats KL it is from 10 to 100, preferably from 15 to 80, with particular preference from 20 to 70, and in particular from 25 to 60  $\mu\text{m}$ .

In accordance with the invention, the surfacer film, topcoat film, basecoat film and clearcoat film may be cured thermally, or thermally and with actinic radiation, depending on their material composition. In accordance with the invention it is of advantage to cure the basecoat film only partly if at all before applying the clearcoat film, and then to cure it together with the clearcoat film (wet-on-wet technique).

Curing may take place after a certain rest period. This period may have a duration of from 30 s to 2 h, preferably from 1 min to 1 h, and in particular from 1 min to 30 min. The rest period is used, for example, for leveling and devolatilization of the coating films or for the evaporation of volatile constituents such as solvents, water or carbon dioxide if the coating material has been applied using supercritical carbon dioxide as solvent (H). The rest period may be shortened and/or assisted by the application of elevated

## 23

temperatures up to 80° C., provided this does not entail any damage or alteration to the coating films, such as premature complete crosslinking, for instance.

The thermal curing has no special features in terms of its method but instead takes place in accordance with the customary and known methods such as heating in a forced-air oven or irradiation with IR lamps. Thermal curing may also take place in stages. Advantageously, it is effected at a temperature of from 50 to 100° C., with particular preference from 80 to 100° C., and in particular from 90 to 100° C., for a period of from 1 min to 2 h, with particular preference from 2 min to 1 h, and in particular from 3 min to 30 min. Where the substrates used have a high capacity to withstand thermal stress, thermal crosslinking may also be conducted at temperatures above 100° C. In general it is advisable in this case not to exceed temperatures of 180° C., preferably 160° C., and in particular 140° C.

Given an appropriate material composition of the coating material, the thermal curing may be supplemented by curing with actinic radiation, it being possible to use UV radiation and/or electron beams. If desired, it may be supplemented by or conducted with actinic radiation from other radiation sources. In the case of electron beams, it is preferred to operate under an inert gas atmosphere. This may be ensured, for example, by supplying carbon dioxide and/or nitrogen directly to the surface of the coating film.

In the case of curing with UV radiation, as well, it is possible to operate under inert gas in order to prevent the formation of ozone.

Curing with actinic radiation is carried out using the customary and known radiation sources and optical auxiliary measures. Examples of suitable radiation sources are high or low pressure mercury vapor lamps, with or without lead doping in order to open up a radiation window of up to 405 nm, or electron beam sources. The arrangement of these sources is known in principle and may be adapted to the circumstances of the workpiece and the process parameters. In the case of workpieces of complex shape such as automobile bodies, the regions not accessible to direct radiation (shadow regions) such as cavities, folds and other structural undercuts may be cured using point, small-area or all-round emitters, in conjunction with an automatic movement means for the irradiation of cavities or edges.

The equipment and conditions for these curing methods are described, for example, in R. Holmes, U.V. and E.B. Curing Formulations for Printing Inks, Coatings and Paints, SITA Technology, Academic Press, London, United Kingdom, 1984.

Curing may take place in stages, i.e., by multiple exposure to light or actinic radiation. This may also be done alternately, i.e., by curing in alternation with UV radiation and electron beams.

Where thermal curing and curing with actinic radiation are employed together (dual cure), these methods may be used simultaneously or in alternation. Where the two curing methods are used in alternation, it is possible, for example, to begin with thermal curing and end with actinic radiation curing. In other cases it may prove advantageous to begin and to end with actinic radiation curing. The skilled worker is able to determine the curing method particularly appropriate to each individual case on the basis of his or her general knowledge in the art, possibly with the aid of simple preliminary experiments.

The multicoat systems ML of the invention have an outstanding profile of properties which is very well balanced in terms of mechanical properties, optical properties, corrosion resistance, and adhesion. Thus the multicoat systems

## 24

ML of the invention have the intercoat adhesion and high optical quality which the market requires and no longer give rise to any problems such as inadequate condensation resistance of the surfacer coats, cracking (mud cracking) in the basecoats, or leveling defects or surface structures in the clearcoats.

In particular, the multicoat system ML of the invention has an outstanding [sic] metallic effect and D.O.I. (distinctiveness of the reflected image) and outstanding surface smoothness. It is stable to weathering, resistant to chemicals and bird droppings, is scratch resistant, and exhibits very good reflow properties.

A further important advantage is the very good overcoatability of the multicoat system ML of the invention, even without sanding. As a result, it can easily be coated with customary and known, highly scratch-resistant coating materials based on organically modified ceramic materials.

Not least, however, it proves to be a very particular advantage that by means of the process of the invention it is possible to produce a multicoat system which is based exclusively on aqueous coating materials.

## EXAMPLES

## Preparation Example 1

## The Preparation of a Dispersion of a Copolymer (A)

A steel reactor as commonly used to prepare dispersions, equipped with a stirrer, a reflux condenser and 3 feed vessels, was charged with 52.563 parts by weight of DI water and this initial charge was heated to 90° C. The first feed vessel was charged with 10.182 parts by weight of acrylic acid, 18.345 parts by weight of methyl methacrylate and 1.493 parts by weight of diphenylethylene. The second feed vessel was charged with 9.914 parts by weight of 25 percent strength ammonia solution. The third feed vessel was charged with 5.25 parts by weight of DI water and 2.253 parts by weight of ammonium peroxodisulfate. With intensive stirring of the initial charge in the steel reactor, the three feed streams were commenced simultaneously. The first and second feed streams were metered in over the course of one hour. The third feed stream was metered in over the course of 1.25 hours. The resultant reaction mixture was held at 90° C. for 4 hours and then cooled to below 40° C. and filtered through a 100  $\mu\text{m}$  GAF bag. The resultant dispersion had a solids content of from 32 to 34% by weight (1 hour, 130° C.) and a free monomer content of less than 0.2% by weight (determined by gas chromatography).

The dispersion (A) was used to prepare a block copolymer (A).

## Preparation Example 2

## The Preparation of a Dispersion of a Block Copolymer (A)

A steel reactor as commonly used to prepare dispersions, equipped with a stirrer, a reflux condenser and a feed vessel, was charged with 51.617 parts by weight of DI water and 9.907 parts by weight of the dispersion from Preparation Example 1 and this initial charge was heated to 90° C. with stirring. Thereafter, a mixture of 9.856 parts by weight of n-butyl methacrylate, 7.884 parts by weight of styrene, 12.661 parts by weight of hydroxyethyl methacrylate and 8.885 parts by weight of ethylhexyl methacrylate was metered in from the feed vessel over the course of six hours. The resultant reaction mixture was stirred at 90° C. for two hours. Subsequently, the resultant dispersion was cooled to below 40° C. and filtered through a 50  $\mu\text{m}$  GAF bag. The dispersion (A) had a solids content of from 41 to 42% by weight (1 hour, 130° C.) and a free monomer content of less than 0.2% by weight (determined by gas chromatography).

## Example 1

The Preparation of a Multicoat System ML of the Invention  
1.1 The Preparation of a Surfacer Comprising the Constituent (A)

## 1.1.1 The Preparation of the Pigment Paste

For the preparation of the surfacer, first of all a pigment paste is prepared from 3.8 parts by weight of lamp black, 32.87 parts by weight of barium sulfate (Blanc Fixe® Super-F), 1.73 parts by weight of talc, 1.04 parts by weight of Additol® XW395 (commercial wetting agent) and 60.56 parts by weight of the dispersion (A) from Preparation Example 2. The mixture was predispersed in a dissolver for ten minutes and then ground on a sand mill to a Hegmann fineness <15 µm. The viscosity of the paste at a shear rate of 100 s<sup>-1</sup> and 23° C. was 160 mPa.s.

## 1.1.2 The Preparation of the Surfacer

The surfacer was prepared by mixing 57.8 parts by weight of the pigment paste from Example 1.1.1 and 30 parts by weight of the dispersion (A) from Preparation Example 2. It had a viscosity of 122 mPa.s at a shear rate of 100 s<sup>-1</sup> and 23° C. The surfacer was adjusted with water to a spray viscosity of 55 mPa.s.

## 1.2 The Preparation of a Metallic Basecoat Material Comprising the Constituent (A) ps 1.2.1 The Preparation of a Color Paste

For the preparation of the metallic basecoat material, first of all a color paste is prepared from 50 parts by weight of the dispersion (A) from Preparation Example 2, 2 parts by weight of Pluriol® P900 (BASF AG), 43 parts by weight of Sicopalgelb® L1100 (BASF AG), 0.4 parts by weight of Agitan® 281 (commercial defoamer; Münzing Chemie GmbH). The mixture was predispersed in a dissolver for ten minutes and then ground in a sand mill to a Hegmann fineness <5 µm. The viscosity of the resultant color paste at a shear rate of 1 000 s<sup>-1</sup> and 23° C. was 424 mpa.s.

For mixing with the metallic paste, 62.8 parts by weight of the dispersion (A) from Preparation Example 2 plus 5 parts by weight of water were added to 37.2 parts by weight of the color paste.

## 1.2.2 The Preparation of a Thixotropic Agent

For the preparation of the metallic basecoat material, the preparation was carried out additionally of a thixotropic agent from 94 parts by weight of DI water, 3.0 parts by weight of Laponite® RD (Solvay Alkali GmbH) and Pluriol® P900 (BASF AG).

## 1.2.3 The Preparation of a Polyester Dispersion

For the preparation of the metallic basecoat material, further, a polyester was prepared in a customary and known manner from 23.23 parts by weight of dimer fatty acid (Pripol® 1009), 10.43 parts by weight of 1,6-hexanediol, 6.28 parts by weight of hexa-hydrophthalic anhydride, 9.9 parts by weight of neopentyl glycol and 10.43 parts by weight of trimellitic anhydride. One part by weight of cyclohexane was used as azeotrope former.

The resultant polyester was dispersed in 17.48 parts by weight of DI water, 18.9 parts by weight of butyl glycol and 2.25 parts by weight of dimethylethanol-amine.

## 1.2.4 The Preparation of a Metallic Paste

For the preparation of the metallic basecoat material, a metallic paste was prepared from 378.7 parts by weight of the thixotropic agent from Example 1.2.2, 74 parts by weight of a commercial polyester (Maprenal® VM 3924), 70 parts by weight of butyl glycol, 334.5 parts by weight of the dispersion (A) from Preparation Example 2, 5 parts by weight of a commercial wetting agent (BYK® 346), 50.6 parts by weight of a commercial aluminum paste (Stapa Hydrolux® 8154), 86 parts by weight of the polyester from Example 1.2.3 and 33 parts by weight of DI water.

The pH of the metallic paste was adjusted to 7.8 using 10% strength dimethylethanolamine solution. The viscosity of the metallic paste was adjusted to 80 mPa.s by further addition of water.

## 1.2.5 The Preparation of the Metallic Basecoat Material

The metallic basecoat material was prepared by mixing the color paste from Example 1.2.1 and the metallic paste from Example 1.2.4 in a weight ratio of 2:10.

## 1.2.6 The Preparation of a Clearcoat Material Comprising the Constituent (A)

To produce the multicoat system ML of the invention, a further preparation conducted was that of a clearcoat material from 100 parts by weight of the dispersion (A) from Preparation Example 2, 5 parts by weight of a commercial crosslinking agent based on tris(alkoxycarbonylamino) triazines (Cylink®2000; CYTEC) and 0.4 parts by weight of Agitan® 281. The mixture, which was of low viscosity, was homogenized using an Ultraturrax. Thereafter, the viscosity at a shear rate of 1.00 s<sup>-1</sup> and 23° C. was 128 mPa.s.

## 1.2.7 The Coating of a Substrate With the Multicoat System ML of the Invention

To produce the multicoat system ML of the invention, customary and known steel test panels were used which had been coated with a commercial electrodeposition coating material.

The test panels were coated pneumatically with the surfacer from Example 1.1. The resultant surfacer film was predried at room temperature for ten minutes and at 80° C. for ten minutes. Thereafter it was baked at 100° C. for 20 minutes and at 130° C. for 20 minutes. This gave a surfacer coat FL with a thickness of 35 µm.

The metallic basecoat material from Example 1.2 was applied pneumatically to the surfacer coat FL. The resultant metallic basecoat film was predried at room temperature for ten minutes and at 80° C. for ten minutes.

The clearcoat material from Example 1.2.6 was applied to the predried metallic basecoat film, after which the resultant clearcoat film was flashed off at room temperature for 15 minutes. Thereafter, the metallic basecoat film and the clearcoat film were baked at 140° C. for 30 minutes (wet-on-wet technique). This gave a metallic basecoat BL with a thickness of 15 µm and a clearcoat KL with a thickness of 35 µm.

The multicoat system ML of the invention produced in this way had an outstanding overall appearance, especially an outstanding metallic effect, an outstanding D.O.I. (distinctiveness of the reflected image), and outstanding surface smoothness. The clearcoat KL was stable to weathering, resistant to chemicals and bird droppings, was scratch resistant, and exhibited very good reflow characteristics.

A further important advantage was the very good over-coatability of the multicoat system ML of the invention, even without sanding. As a result, it was easy to coat the clearcoat KL with customary and known, highly scratch-resistant coatings based on organically modified ceramic materials.

What is claimed is:

1. A multicoat color and/or effect coating system for a primed or unprimed substrate, comprising, at least one coat being produced from a coating material comprising at least one constituent (A) made by free-radical polymerization of
  - a) at least one olefinically unsaturated monomer and
  - b) at least one olefinically unsaturated monomer different than the olefinically unsaturated monomer (a) and of the general formula I



(I),

## 27

in which the radicals R<sup>1</sup>, R<sup>2</sup>, R<sup>3</sup> and R<sup>4</sup> each independently of one another are hydrogen atoms or substituted or unsubstituted alkyl, cycloalkyl, alkylcycloalkyl, cycloalkylalkyl, aryl, alkylaryl, cycloalkylaryl, arylalkyl or arylcycloalkyl radicals, with the proviso that at least two of the variables R<sup>1</sup>, R<sup>2</sup>, R<sup>3</sup> and R<sup>4</sup> are substituted or unsubstituted aryl, arylalkyl or arylcycloalkyl radicals;

in an aqueous medium.

2. A process for producing a multicoat color and/or effect coating system ML on a substrate, comprising applying at least one coating composition to the substrate and curing the at least one coating composition to provide a cured coat, wherein the at least one coating composition comprises at least one constituent (A) made by free-radical polymerization of

- a) at least one olefinically unsaturated monomer,
- b) at least one olefinically unsaturated monomer different than the olefinically unsaturated monomer (a) and of the general formula I



in which the radicals R<sup>1</sup>, R<sup>2</sup>, R<sup>3</sup> and R<sup>4</sup> each independently of one another are hydrogen atoms or substituted or unsubstituted alkyl, cycloalkyl, alkylcycloalkyl, cycloalkylalkyl, aryl, alkylaryl, cycloalkylaryl, arylalkyl or arylcycloalkyl radicals, with the proviso that at least two of the variables R<sup>1</sup>, R<sup>2</sup>, R<sup>3</sup> and R<sup>4</sup> are substituted or unsubstituted aryl, arylalkyl or arylcycloalkyl radicals;

in an aqueous medium.

3. The multicoat system of claim 1, characterized in that the constituent (A) is obtained by

- (i) subjecting at least one monomer (a) and at least one monomer (b) to free-radical polymerization in an aqueous medium to provide a reaction product, and then
- (ii) reacting the resultant reaction product with at least one further monomer (a) under free-radical conditions.

4. The multicoat system of claim 1, characterized in that the aryl radicals R<sup>1</sup>, R<sup>2</sup>, R<sup>3</sup> and/or R<sup>4</sup> of the monomer (b) comprise phenyl or naphthyl radicals.

5. The multicoat system of claim 1, characterized in that the substituents in radicals R<sup>1</sup>, R<sub>2</sub>, R<sub>3</sub> and/or R<sup>4</sup> of the compound (b) are electron-donating or electron-withdrawing atoms or organic radicals.

6. The multicoat system of claim 1, wherein monomers (a) comprise at least one member selected from

- a1) (meth)acrylic esters which are essentially free from acid groups;
- a2) monomers which carry per molecule at least one group selected from hydroxyl group, amino group, alkoxyethylamino group or imino group and are essentially free from acid groups;
- a3) monomers which carry per molecule at least one acid group which can be converted into the corresponding acid anion group;
- a4) vinyl esters of alpha-branched monocarboxylic acids having 5 to 18 carbon atoms in the molecule;
- a5) reaction products of acrylic acid and/or methacrylic acid with the glycidyl ester of an alpha-branched monocarboxylic acid having 5 to 18 carbon atoms per molecule;
- a6) cyclic and/or acyclic olefins;

## 28

- a7) (meth)acrylamides;
- a8) monomers containing epoxide groups;
- a9) vinylaromatic hydrocarbons;
- a10) nitriles;
- a11) vinyl compounds, especially vinyl halides and/or vinylidene dihalides, N-vinylpyrrolidone, vinyl ethers and/or vinyl esters;
- a12) allyl compounds, especially allyl ethers and allyl esters;
- a13) polysiloxane macromonomers having a number-average molecular weight Mn of from 1000 to 40 000 and having on average from 0.5 to 2.5 ethylenically unsaturated double bonds per molecule; and/or
- a14) acryloxy silane-containing vinyl monomers, prepared by reacting hydroxyl-functional silanes with epichlorohydrin and then reacting the reaction product with (meth)acrylic acid and/or with hydroxyalkyl and/or hydroxycycloalkyl esters of (meth)acrylic acid (monomers a2), and mixtures thereof.

7. The multicoat system of claim 1, characterized in that the coating material further comprises at least one of the following constituents:

- A') at least one binder having at least one functional group (afg) which is able to undergo thermal crosslinking reactions with complementary functional groups (bfg) in the crosslinking agent (B);
- B) at least one crosslinking agent having at least two functional groups (bfg) which are able to undergo thermal crosslinking reactions with complementary functional groups (afg) in the constituent (A'),
- C) at least one constituent which is crosslinkable with actinic radiation,
- D) at least one photoinitiator,
- E) at least one thermal crosslinking initiator,
- F) at least one reactive diluent curable thermally and/or with actinic radiation,
- G) at least one coatings additive,
- H) at least one organic solvent, ps and mixtures thereof.

8. A process of coating an article selected from automotive OEM finishing, automotive refinishing, industrial coating, coil coating, container coating, the coating of plastics, and furniture coating, comprising applying the multicoat coating system of claim 1 to at least one surface of the article and curing it.

9. A coated article comprising at least one multicoat system of claim 1.

10. The multicoat color and/or effect coating system of claim 1 wherein the at least one coat of the coating system is at least one coat selected from the group consisting of a surfacer coat FL which absorbs mechanical energy, a color and/or effect topcoat DL, a color and/or effect basecoat BL, a clearcoat KL, and combinations thereof.

11. The multicoat color and/or effect coating system of claim 10 wherein the coating system consists of

- (1) a surfacer coat FL which absorbs mechanical energy, and
- (2) a color and/or effect topcoat DL, lying above one another in the stated sequence.

12. The multicoat color and/or effect coating system of claim 11 wherein both coat FL and topcoat DL are produced from a coating material comprising at least one constituent (A).

13. The multicoat color and/or effect coating system of claim 10 wherein the coating system consists of

**29**

(1) a surfacer coat FL which absorbs mechanical energy,  
 (2) a color and/or effect basecoat BL, and  
 (3) a clearcoat KL,  
 lying above one another in the stated sequence.

14. The multicoat color and/or effect coating system of claim 13 wherein at least two of coat FL, basecoat BL and clearcoat KL are produced from a coating material comprising at least one constituent (A).

15. The multicoat color and/or effect coating system of claim 14 wherein at all three of coat FL, basecoat BL and clearcoat KL are produced from a coating material comprising at least one constituent (A).

16. The multicoat color and/or effect coating system of claim 10 wherein the coating system consists of

- (1) a color and/or effect basecoat BL and  
 (2) a clearcoat KL,

lying above one another in the stated sequence.

17. The multicoat color and/or effect coating system of claim 16 wherein both basecoat BL and clearcoat KL are produced from a coating material comprising at least one constituent (A).

18. The multicoat color and/or effect coating system of claim 1 wherein at least two of the radicals R1, R2, R3 and R4 are substituted with substituted or unsubstituted aryl radicals.

19. The process of claim 2 further comprising

- (I) applying a surfacer coating material to a substrate to provide a surfacer film,  
 (II) curing the surfacer film to give a surfacer coat FL,  
 (III) preparing a solid-color topcoat film by applying a solid-color coating material to the surfacer coat FL, and  
 (IV) curing the solid-color topcoat film to give a solid-color topcoat DL,

wherein both of the applied coating materials comprise at least one constituent (A) in aqueous medium.

20. The process of claim 2 further comprising

- (I) preparing a basecoat film by applying a basecoat coating material to the substrate,

**30**

(II) drying the basecoat film,  
 (III) preparing a clearcoat film by applying a clearcoat coating material to the basecoat film, and  
 (IV) jointly curing the basecoat film and the clearcoat film to give the basecoat BL and the clearcoat KL, wherein both of the applied coating materials comprise at least one constituent (A) in aqueous medium.

21. The process of claim 2 further comprising

- (I) preparing a surfacer film by applying a surfacer coating material to a substrate,  
 (II) curing the surfacer film to give the surfacer coat FL,  
 (III) preparing a basecoat film by applying a basecoat coating material to the surfacer coat FL,  
 (IV) drying the basecoat film,  
 (V) preparing a clearcoat film by applying a clearcoat coating material to the basecoat film, and  
 (VI) jointly curing the basecoat film and the clearcoat film to give the basecoat BL and the clearcoat KL,

wherein at least two of the coating materials applied comprise at least one constituent (A) in aqueous medium.

22. The process of claim 21 wherein the three applied coating materials comprise at least one constituent (A) in aqueous medium.

23. New) The multicoat system of claim 4, characterized in that the aryl radicals R<sup>1</sup>, R<sup>2</sup>, R<sup>3</sup> and/or R<sup>4</sup> of the monomer (b) comprise phenyl radicals.

24. The multicoat system of claim 5, wherein the substituents in radicals R<sup>1</sup>, R<sup>2</sup>, R<sup>3</sup> and/or R<sup>4</sup> of the compound (b) are at least one or more groups selected from halogen atoms, nitrile, nitro, partially or fully halogenated alkyl, cycloalkyl, alkylcycloalkyl, cycloalkylalkyl, aryl, alkylaryl, cycloalkylaryl, arylalkyl and arylcycloalkyl radicals; aryloxy, alkyloxy and cycloalkyloxy radicals; arylthio, alkythio and cycloalkylthio radicals; hydroxyl groups, primary, secondary and/or tertiary amino groups, and mixtures thereof.

\* \* \* \* \*